

Oct. 27, 1936.

A. HOCHE

2,058,791

PULP PROCESS

Original Filed Nov. 20, 1934



INVENTOR  
*Adam Hoché*  
BY  
*Lyman E. Dodge*  
ATTORNEY

## UNITED STATES PATENT OFFICE

2,058,791

## PULP PROCESS

Adam Hoche, Brooklyn, N. Y.

Application November 20, 1934, Serial No. 753,798  
Renewed March 18, 1936

3 Claims. (Cl. 92—9)

This invention relates to cellulose fibre, particularly to the separation thereof from bodies consisting largely thereof associated with undesired natural substances.

Those skilled in the art of making cellulose pulp, that is, the separation of cellulose fibres from bodies consisting largely thereof associated with undesired or deleterious substances, are fully aware that the present day processes include many steps, which require costly equipment, are slow in operation, and, due to the necessary agitation of the fibre and the subjection thereof to powerful chemical substances for protracted periods, result in a pulp or fibre which is both short and weak. A further disadvantage with present processes is the low yield.

Applicant, realizing the deficiencies in present day processes, after protracted study, experimentation, analysis and testing arrived at the conclusion that a proper process for the recovery of cellulose fibres, must be one in which, the fibre is subjected to the least possible mechanical agitation or handling; to the lowest possible temperature; treated for the shortest possible time; subjected to a chemical substance or substance most active in action upon the foreign or deleterious or undesired substances associated with the fibre, and least active or injurious to the fibre itself; and, further, that the process should preferably be such that the number of steps is reduced to a minimum, preferably substantially one, to the end that separation and bleaching be accomplished in one treatment.

With this end in view, applicant has devised a process for the separation of cellulose fibre from associated undesired natural substances which is, in effect, a one step process. This process is carried out without mechanical agitation; at room temperature, save for any increased temperature due to the reacting masses; necessitates an extremely short exposure of the fibre to the chemicals used; includes the use of chemicals which are extremely active toward the undesired and deleterious substances and comparatively inert, in the concentrations used, toward the cellulose; and substantially separates the deleterious substances and bleaches in one treatment, which completes the process save for a necessary separation of the chemicals used from the treated material and a subsequent water wash of the material to remove the last traces of chemicals and soluble impurities from the cellulose pulp.

In order to better describe the new process applicant has selected a specific form of apparatus merely to illustrate the carrying out of the process.

In describing the invention in detail and the particular form of apparatus selected to illustrate the invention, reference is had to the accompanying drawing in which like characters of reference

designate like parts throughout the several views, and in which:

Figure 1 is a side elevational view with some parts broken away to more clearly show the construction, of an apparatus by which applicant's process may be carried out; Fig. 2 is a top plan view of the apparatus as shown in Fig. 1.

In carrying out the process, applicant selects a suitable cellulose fibre carrying mass, such as wood chips, sisal, hemp, bagasse or the like, in fact any of the ordinary and well known source materials.

The selected material is placed in a vessel of suitable form, size and material and equipped with the obvious accessories for facilitating the treatment. In general, any vessel of the general form of a tank is suitable. The material is preferably placed somewhat loosely in the tank, to the end that the treating solution may readily penetrate to every particle.

In Figure 1 applicant has illustrated vessels 1, 2, 3, 4 and 5 which may be considered as any ordinary well known type of vessel of the form shown which is formed of an acid resisting material, preferably glass.

Applicant puts into each of the vessels 1 to 5 inclusive selected material about up to the line 6.

Each of the vessels is provided with a stopper, as 7, formed with two orifices therethrough. The stopper of vessel 1 has a tube 8 of acid resisting material, preferably glass, passed through one of the orifices and a filling and safety tube 9 of similar material passed through the other orifice in the stopper 7. Each of the other vessels has a long tube as 10 passing through the stopper of the vessel which long tube reaches nearly to the bottom of the vessel; and another short tube 11 comparable with the tube 8 which passes through the orifice in the stopper and terminates shortly below the stopper.

The short tube, as 8, of one vessel is connected to the long tube, as 10, of the next succeeding vessel by any suitable and appropriate means such as by a flexible tube 12 made preferably of an acid resisting material such as caoutchouc or rubber.

Onto the material of vessel 1, applicant flows directly while the stopper 7 is partially removed, or by way of the filling tube 9, a solution of water and nitric acid mixed to a concentration of from 1° to 45° Baumé and in addition adds a starch or saccharose such as cane sugar or molasses thereto. The cane sugar is added in the proportion of about 5 pounds of cane sugar to 1 ton of wood chips, but this may be decreased to about 1 pound in some cases and in others increased to 8 pounds depending upon the quantity of substances in the fibre mass capable of forming oxalic acid, or the rapidity to which it is desired for the reaction to proceed.

The contents of vessel 1 are made exactly in accordance with the disclosure of my copending application for Pulp process, Serial No. 751,255, filed November 2, 1934.

5 The contents of vessels 2, 3, 4 and 5 are each alike and consist of wood chips or other suitable fibre bearing mass together with water solution of sulphuric acid of 1% to 10% concentration.

10 The reaction between the materials of vessel 1 starts at ordinary room temperature and at ordinary atmospheric pressure. As reaction proceeds the contents of vessel 1 become somewhat heated and a certain amount of distillation takes place through the tubes 8, 12 and 10.

15 The products thus distilled issue from the lower end of the tube 10 and bubble through the liquid of vessel 2. As the reaction proceeds there may be further transfer from vessel 2 to vessel 3, and from 3 to 4, and from 4 to 5, but usually the 20 major absorption takes place in vessel 2. The reaction in vessel 2 is allowed to proceed until the fibre bearing mass therein has been so acted upon, that it is in condition to be water washed, whereupon the contents of vessel 2 are removed, 25 the surplus liquid drawn out by any appropriate means such as by a centrifuge, and then the mass water washed in any suitable and appropriate manner. In case a centrifuge is used to remove the acid liquor, then the mass may be 30 water washed in the centrifuge.

The product obtained is a cellulose fibre of great strength and of a color such that it requires no bleaching.

35 The process gives a very high yield of fibre and the fibre is strong and suitable for use in those processes which require a strong white cellulose fibre.

40 The exact chemical reactions are not, perhaps, thoroughly understood, but it is believed that the reaction in vessel 1 in which there is a dilute solution of nitric acid together with a fibre mass and a carbohydrate, generates oxalic acid and some oxides of nitrogen. It is believed that the 45 oxalic acid is the active disintegrating agent and some passes over from vessel 1 to vessel 2 and serves to disintegrate the fibre mass so as to separate the cellulose therefrom. At the same time, the dilute solution of sulphuric acid in vessel 2 tends to form a sugar with some of the substances present in the fibre mass and this sugar reacts with the oxides of nitrogen which bubbles through the liquid to further form an oxalic acid which further acts to disintegrate the fibre mass.

55 The strength of acid used in vessel 1 and the strength of acid used in vessels 2 to 5 inclusive depends upon the resistance of the material used. If the material is very resistant and rapidity is desired, then a strong acid solution is used in vessel 1 and a strong acid solution in vessels 2 to 5, inclusive.

60 The process is particularly noteworthy because it produces a fibre which is rich in oxy cellulose and is therefore particularly useful in the making of cellulose esters.

65 The process is inexpensive because only about 5 to 10% of the nitric acid in vessel 1 is consumed by a single treatment of a fibre bearing mass. The remainder is recovered by, for example, the separation at the centrifuge as explained in 70 the application hereinafter referred to, and may be used again by bringing it up to proper strength.

After the material in vessel 2 has been brought to the proper condition for washing the connection from vessel 1 may be made directly to

vessel 3; and after the material in vessel 3 has been suitably treated connection in the same manner may be made to vessel 4 and then to vessel 5. In case connection is made directly from vessel 1 to vessel 3, applicant would connect a fresh vessel with vessel 5, that is, applicant prefers to always have at least 4 vessels, as 5 to 5 inclusive, connected to a vessel such as 1 in which the reaction is proceeding, so that every last particle of distillate is absorbed even if the 10 adjoining vessel as 2 has practically completely reacted so that a large amount of distillation takes place from 2 to 3.

This process may be considered as an extension of the process of my prior application hereinbefore referred to as the vessel 1 is used to carry out the process exactly as described in my prior application. The remaining vessels are used to save and preserve that which otherwise would be a loss in carrying out the process in 15 vessel 1.

20 Having described the principle and mode of operation of my invention and a particular application thereof and a specific apparatus by which my process may be carried out, I desire 25 to have it understood that the specific apparatus selected is merely illustrative and does not exhaust the possible apparatus forms by which the underlying principles of my invention may be exemplified.

30 What I claim as new and desire to secure by Letters Patent of the United States, is:

1. A process of separating cellulose fibre from a fibre mass admixed with undesired other natural substances and simultaneously bleaching it 35 which consists in substantially covering the mass with a water solution of 1% to 10% of sulphuric acid, bubbling through that solution products distilled from a reaction taking place between a fibre mass admixed with undesired other natural 40 substances and dilute nitric acid, and then separating the liquids from the solids and washing with water until substantially acid free.

2. A process of separating cellulose fibre from a fibre mass admixed with undesired other natural substances and simultaneously bleaching it 45 which consists in substantially covering the mass with a water solution of 1% to 10% of sulphuric acid, bubbling through that solution products distilled from a reaction taking place between a 50 fibre mass admixed with undesired other natural substances, dilute nitric acid and substances selected from the group comprising saccharose, starch, and molasses, and then separating the liquids from the solids and washing with water 55 until substantially acid free.

3. A process of separating cellulose fibre from a fibre mass admixed with undesired other natural substances and simultaneously bleaching it which consists in substantially covering the mass with a water solution of 1% to 10% of sulphuric acid, bubbling through the solution products distilled from a reaction taking place between a fibre mass admixed with undesired other natural 60 substances, dilute nitric acid of a concentration from 1° to 45° Baumé at room temperature and at ordinary atmospheric pressure with absence of agitation and about 1 to 8 pounds of a substance selected from the group comprising cane sugar, starch and molasses to two thousand pounds of said fibre mass, and then separating the liquids from the solids and washing with water until 65 substantially acid free.

70 ADAM HOCHE.